



US009539703B2

(12) **United States Patent**  
**Bao**

(10) **Patent No.:** **US 9,539,703 B2**  
(b5) **Date of Patent:** **\*Jan. 10, 2017**

(54) **CARBONATE PCD WITH A DISTRIBUTION OF SI AND/OR AL**

(71) Applicant: **SMITH INTERNATIONAL, INC.**,  
Houston, TX (US)

(72) Inventor: **Yahua Bao**, Orem, UT (US)

(73) Assignee: **Smith International, Inc.**, Houston, TX (US)

(\*) Notice: Subject to any disclaimer, the term of this patent is extended or adjusted under 35 U.S.C. 154(b) by 0 days.

This patent is subject to a terminal disclaimer.

(21) Appl. No.: **14/213,721**

(22) Filed: **Mar. 14, 2014**

(65) **Prior Publication Data**

US 2014/0259962 A1 Sep. 18, 2014

**Related U.S. Application Data**

(60) Provisional application No. 61/801,182, filed on Mar. 15, 2013.

(51) **Int. Cl.**

**B24D 3/00** (2006.01)  
**B24D 3/02** (2006.01)  
**B24D 11/00** (2006.01)  
**B24D 18/00** (2006.01)  
**C09K 3/14** (2006.01)  
**B24D 99/00** (2010.01)

(52) **U.S. Cl.**

CPC ..... **B24D 18/0009** (2013.01); **B24D 99/005** (2013.01)

(58) **Field of Classification Search**

USPC ..... 51/309, 308, 293, 307  
See application file for complete search history.

(56) **References Cited**

**U.S. PATENT DOCUMENTS**

|                 |         |                    |
|-----------------|---------|--------------------|
| 5,624,756 A     | 4/1997  | Ueda et al.        |
| 6,068,913 A     | 5/2000  | Cho et al.         |
| 8,323,367 B1    | 12/2012 | Bertagnolli et al. |
| 8,342,269 B1    | 1/2013  | Bertagnolli et al. |
| 8,353,974 B2    | 1/2013  | Cooley et al.      |
| 8,365,846 B2    | 2/2013  | Dourfaye et al.    |
| 2005/0050801 A1 | 3/2005  | Cho et al.         |
| 2006/0060391 A1 | 3/2006  | Eyre et al.        |

(Continued)

**OTHER PUBLICATIONS**

"Drill bits comprising superabrasive cutting elements formed from polycrystalline diamond and methods of forming same", IP.com Prior Art Database Disclosure No. IPCOM000158151D, Sep. 17, 2007.

(Continued)

*Primary Examiner* — James McDonough

(57) **ABSTRACT**

A method for making a carbonate polycrystalline diamond body includes combining a first quantity of diamond with a first quantity of magnesium carbonate to form a first layer for forming a working surface, and combining a second quantity of magnesium carbonate to form a second layer adjacent to the first layer, forming an assembly. The method includes placing a quantity of silicon or aluminum in or adjacent to at least a portion of the assembly and sintering the assembly including the silicon or aluminum at high pressure and high temperature, causing the silicon or aluminum to infiltrate at least one layer of the assembly.

**12 Claims, 8 Drawing Sheets**



(56)

**References Cited**

U.S. PATENT DOCUMENTS

2010/0242375 A1\* 9/2010 Hall ..... B22F 3/14  
51/307  
2010/0243337 A1 9/2010 Scott  
2011/0023375 A1 2/2011 Sani et al.  
2011/0031034 A1 2/2011 Digiovanni et al.  
2011/0061942 A1 3/2011 Digiovanni  
2011/0252713 A1 10/2011 Chakraborty et al.  
2011/0297453 A1 12/2011 Mukhopadhyay et al.  
2012/0102843 A1 5/2012 Chakraborty et al.  
2012/0241224 A1\* 9/2012 Qian ..... B22F 5/00  
175/428  
2013/0043078 A1 2/2013 Qian et al.

OTHER PUBLICATIONS

Arima, et al., "Diamond nucleation and growth by reduction of carbonate melts under high-pressure and high-temperature conditions", Geology, vol. 30 (8), 2002, p. 691-694.

International Search Report and Written Opinion issued in PCT/US2014/027770 on Jul. 10, 2014, 17 pages.

First Office Action issued in related CN application 201480016011.7 on May 25, 2016, 17 pages.

\* cited by examiner

FIG. 1



FIG. 2a



FIG. 3a



FIG. 2b



FIG. 2d



FIG. 2c



FIG. 3b



FIG. 4



FIG. 5



FIG. 6



FIG. 7



FIG. 8



FIG. 9



FIG. 10



## 1

CARBONATE PCD WITH A DISTRIBUTION  
OF SI AND/OR ALCROSS-REFERENCE TO RELATED  
APPLICATION

This application claims the benefit of U.S. Provisional Patent Application Ser. No. 61/801,182 filed on Mar. 15, 2013, entitled, "CARBONATE PCD WITH A DISTRIBUTION OF SI AND/OR AL ELEMENTS," which is incorporated herein by reference in its entirety.

## BACKGROUND

Ultra-hard materials are often used in cutting tools and rock drilling tools. Polycrystalline diamond material is one such ultra-hard material, and is known for its good wear resistance and hardness. To form polycrystalline diamond, diamond particles are sintered at high pressure and high temperature (HPHT sintering), as for example at pressure equal to or greater than 50 kbar and temperature equal or great than 1350° C., to produce an ultra-hard polycrystalline structure. A catalyst material is added to the diamond particle mixture prior to HPHT sintering and/or infiltrates the diamond particle mixture during HPHT sintering in order to promote the intergrowth of the diamond crystals during HPHT sintering, to form the polycrystalline diamond (PCD) structure. Metals conventionally employed as the catalyst are selected from the group of solvent metal catalysts of Group VIII of the Periodic table, including cobalt, iron, and nickel, and combinations and alloys thereof. After HPHT sintering, the resulting PCD structure includes a network of interconnected diamond crystals or grains bonded to each other, with the catalyst material occupying the interstitial spaces or pores between the bonded diamond crystals. The diamond particle mixture may be HPHT sintered in the presence of a substrate, to form a PCD compact bonded to the substrate. The substrate may also act as a source of the metal catalyst that infiltrates into the diamond particle mixture during sintering.

The amount of catalyst material used to form the PCD body represents a compromise between desired properties of strength, toughness, and impact resistance versus hardness, wear resistance, and thermal stability. While a higher metal catalyst content generally increases the strength, toughness, and impact resistance of the resulting PCD body, this higher metal catalyst content also decreases the hardness and wear resistance as well as the thermal stability of the PCD body. This trade-off makes it difficult to provide a PCD having desired levels of hardness, wear resistance, thermal stability, strength, impact resistance, and toughness to meet the service demands of particular applications, such as in cutting and/or wear elements used in subterranean drilling devices.

Thermal stability can be particularly relevant during wear or cutting operations. Conventional PCD bodies may be vulnerable to thermal degradation when exposed to elevated temperatures during cutting and/or wear applications. This vulnerability results from the differential that exists between the thermal expansion characteristics of the metal catalyst disposed interstitially within the PCD body and the thermal expansion characteristics of the intercrystalline bonded diamond. This differential thermal expansion is known to start at temperatures as low as 400° C., and can induce thermal stresses that are detrimental to the intercrystalline bonding of diamond and that eventually result in the formation of cracks that can make the PCD structure vulnerable to failure. Accordingly, such behavior is not desirable.

## 2

Another form of thermal degradation known to exist with conventional PCD materials is one that is also related to the presence of the metal catalyst in the interstitial regions of the PCD body and the adherence of the metal catalyst to the diamond crystals. Specifically, the metal catalyst is known to cause an undesired catalyzed phase transformation in diamond (converting it to carbon monoxide, carbon dioxide, or graphite) with increasing temperature, thereby limiting the temperatures at which the PCD body may be used.

To improve the thermal stability of the PCD material, a carbonate catalyst has been used to form the PCD. PCD formed with a carbonate catalyst is referred to hereinafter as "carbonate PCD." The carbonate catalyst is mixed with the diamond particles prior to sintering, and promotes the growth of diamond grains during sintering. When a carbonate catalyst is used, the diamond remains stable in polycrystalline diamond form with increasing temperature, rather than being converted to carbon dioxide, carbon monoxide, or graphite. Thus the carbonate PCD is more thermally stable than PCD formed with a metal catalyst.

However, the carbonate catalyst itself is subject to a decomposition reaction with increasing temperature, converting to a metal oxide. The carbonate may be released as CO<sub>2</sub> gas, causing outgassing of the carbonate PCD material. This outgassing can cause volume expansion and undesirable voids, bubbles, or films on adjacent surfaces, leading to imperfections and cracks in the ultra-hard material as well as decreased wear resistance.

## SUMMARY

This summary is provided to introduce a selection of concepts that are further described below in the detailed description. This summary is not intended to identify key or essential features of the claimed subject matter, nor is it intended to be used as an aid in limiting the scope of the claimed subject matter.

In some embodiments, a carbonate polycrystalline diamond body having a working surface opposite a non-working surface includes a first layer having a material microstructure including a plurality of bonded-together diamond crystals and interstitial spaces therebetween, a portion of the interstitial spaces being occupied by a first quantity of magnesium carbonate, and the first layer defining the working surface, and a second layer adjacent to the first layer at a location opposite the working surface, the second layer having a material microstructure including a plurality of bonded-together diamond crystals and interstitial spaces therebetween, a portion of the interstitial spaces being occupied by a second quantity of magnesium carbonate greater than the first quantity. At least a quantity of at least one of silicon, aluminum, or a combination thereof is in at least one of the first layer or the second layer.

In some embodiments, a method for making a carbonate polycrystalline diamond body includes combining a first quantity of diamond particles with a first quantity of magnesium carbonate to form a first layer for forming a working surface and combining a second quantity of diamond particles with a second quantity of magnesium carbonate to form a second layer, the second quantity of magnesium carbonate being greater than the first quantity of magnesium carbonate, the second layer being formed adjacent to the first layer, and the first layer and the second layer together forming an assembly. A quantity of at least one of silicon or aluminum is placed in or adjacent to at least a portion of the assembly. The assembly including the quantity of at least one of silicon or aluminum is sintered at high pressure and

high temperature, causing the silicon or aluminum to infiltrate at least one layer of the assembly.

#### BRIEF DESCRIPTION OF THE DRAWINGS

Embodiments of the present disclosure are described with reference to the following figures.

FIG. 1 illustrates a schematic view of a material microstructure of a carbonate polycrystalline diamond material according to an embodiment (where the dimensions may be exaggerated and thus the drawing may not be to scale, for clarity).

FIG. 2a illustrates a cross-sectional view of can including an assembly having a first layer and a second layer including a distribution of a Si and/or Al compound, prior to HPHT sintering, according to an embodiment.

FIG. 2b illustrates a cross-sectional view of a can including an assembly having a first layer, a second layer, and a third layer including a distribution of a Si and/or Al compound, prior to HPHT sintering, according to an embodiment.

FIG. 2c illustrates a cross-sectional view of a can including an assembly having a first layer, a second layer including a distribution of a Si and/or Al compound, and a substrate, prior to HPHT sintering, according to an embodiment.

FIG. 2d illustrates a cross-sectional view of a can including an assembly having a first layer, a second layer, a third layer including a distribution of a Si and/or Al compound, and a substrate prior to HPHT sintering, according to an embodiment.

FIG. 3a illustrates a perspective view of the diamond compact incorporating a carbonate polycrystalline diamond body after HPHT sintering of the assembly illustrated in FIG. 2a, including a first layer or working surface, and a second layer or non-working surface, according to an embodiment.

FIG. 3b illustrates a perspective view of the diamond compact incorporating a carbonate polycrystalline diamond body after HPHT sintering of the assembly illustrated in FIG. 2c, including a first layer or working surface, a second layer or non-working surface, and a substrate, according to an embodiment.

FIG. 4 is a flowchart illustrating a method of forming a carbonate polycrystalline diamond body incorporating a distribution of a Si and/or Al compound, according to an embodiment.

FIG. 5 illustrates a perspective view of a drag bit incorporating the diamond compact element of FIG. 3a or 3b after subsequent heat-treatment.

FIG. 6 is an X-ray diffraction pattern graph for a carbonate polycrystalline diamond layer including less than 0.2 wt % silicon, heated-treated to 1200° C. under vacuum.

FIG. 7 is an X-ray diffraction pattern graph for a carbonate polycrystalline diamond showing a layer including less than 0.2 wt % silicon, and a layer including approximately 1.5 wt % silicon, heated-treated to 900° C. under vacuum, according to an embodiment.

FIG. 8 is a graph of the distribution of Silicon along the thickness of a PCD body including a 0.5 wt % SiC compound mixed with diamond particles of a second layer of the PCD body, according to an embodiment.

FIG. 9 is a graph of the distribution of Silicon along the thickness of a PCD body including a 1.5 wt % SiO<sub>2</sub> compound mixed with the diamond particles of a second layer of the PCD body, according to an embodiment.

FIG. 10 is a graph comparatively demonstrating the distribution of Magnesium along the thickness of a PCD

body including a MgCO<sub>3</sub> catalyst infiltrating the assembly from the second layer of the PCD body versus from the first layer of the PCD body, according to an embodiment.

#### DETAILED DESCRIPTION

The present disclosure relates to ultra-hard materials, and more particularly in some embodiments, to ultra-hard materials formed with a carbonate catalyst having controlled thermal decomposition, and methods for forming the same. For clarity, as used herein, the term “PCD” refers to conventional polycrystalline diamond that has been formed with the use of a metal catalyst during an HPHT sintering process, forming a microstructure of bonded diamond crystals with the catalyst material occupying the interstitial spaces or pores between the bonded diamond crystals. The term “carbonate PCD” refers to PCD formed with a carbonate catalyst, forming a microstructure of bonded diamond crystals with the carbonate catalyst material occupying the interstitial spaces or pores between the bonded diamond crystals.

A region of a carbonate PCD material 10 is schematically illustrated in FIG. 1. The carbonate PCD material 10 has a polycrystalline microstructure including multiple diamond grains or crystals 14 bonded to each other, with interstitial spaces or pores 18 between the diamond crystals. This polycrystalline microstructure is formed by subjecting diamond particles to an HPHT sintering process in the presence of a carbonate catalyst. In some embodiments, the HPHT sintering process includes applying a pressure of about 50 kbar or greater, and a temperature of greater than 1350° C. In other embodiments, the HPHT sintering process includes applying a pressure of about 65 kbar or greater, and a temperature of greater than 1800° C. At this temperature and pressure, the carbonate catalyst material melts and infiltrates the diamond particles mixture. The catalyst promotes the direct bonding of diamond crystals during the HPHT sintering process, forming carbonate PCD. The result is a carbonate PCD material with the carbonate catalyst material 16 occupying the interstitial spaces 18 between the diamond crystals 14 (referred to hereinafter as “grains”). In some embodiments, the diamond grains 14 in the carbonate PCD material have a size in the range of 1 to 20 microns.

In some embodiments, a carbonate PCD body is formed by subjecting an ultra-hard diamond element such as a volume of diamond particles to an HPHT sintering process in the presence of a carbonate catalyst such as magnesium carbonate (MgCO<sub>3</sub>). Various embodiments of the assemblies of the various layers constituting a carbonate PCD body prior to sintering are shown in FIGS. 2a-2d. In these embodiments, the carbonate PCD body 20 is formed by mixing the diamond particles with the carbonate catalyst before HPHT sintering to create the carbonate PCD body. The formed carbonate PCD body 20 is subsequently heat-treated under vacuum or at atmospheric pressure at temperature of approximately 1100° C. to 1200° C. to convert a portion of the carbonate catalyst into an oxide, while releasing a gas. In embodiments including an MgCO<sub>3</sub> carbonate catalyst, the oxide is magnesium oxide (MgO), while the gas is carbon dioxide (CO<sub>2</sub>).

With continued reference to FIGS. 2a-2d, the carbonate PCD body 20 of these embodiments is formed in a refractory can or container 28 including a series of layers 22, 24, and optionally layer 26 and/or substrate 27. In some embodiments, the series of layers includes a first layer 22 including a working surface 23 defined at one surface of the first layer 22. In most embodiments, the first layer 22 is subdivided

into at least two layers prior to HPHT sintering, where at least one layer includes a diamond particle mixture, and at least a second layer includes a carbonate catalyst layer adjacent to the working surface side 23 of the first layer 22 at the diamond particle mixture layer. In some embodiments, the series of layers includes second layer 24 including a non-working surface 21 defined at one surface of the second layer 24 at an opposite surface of the working surface 23. The second layer 24 includes a diamond particle mixture. In some embodiments, the series of layers includes an optional third layer 26, that may be adjacent to the second layer 24 or to the first layer 22, and may include a diamond particle mixture, a carbonate catalyst, or any combination thereof. In some embodiments, the series of layers may optionally include a substrate 27 adjacent to the non-working surface 21 during HPHT sintering. The refractory can or container 28 contains the series of layers 22, 24, and optionally layer 26 and/or substrate 27, and protects them from the surrounding environment while safely containing the HPHT sintering process. The refractory can or container 28 may also have a lid 30 which fits over the top end of the refractory can or container 28. The refractory can or container 28 and lid 30 are formed from a refractory metal such as niobium, molybdenum, or tantalum.

Generally, when a non-metal catalyst such as a carbonate is used in forming a carbonate PCD body, the diamond remains stable while being converted to polycrystalline diamond form during HPHT sintering with increasing temperatures up to 1200° C., without being converted to carbon dioxide, carbon monoxide, or graphite. However, during subsequent heat-treatment cycles of the formed carbonate PCD under atmospheric pressure or vacuum (after HPHT sintering) for the purpose of decomposing the carbonate catalyst, the PCD may develop cracks at temperatures between 800° C. and 1200° C., and may be subject to graphitization. This threshold temperature of 1200° C. is very close to the thermally stable temperature of PCD under vacuum. In some embodiments, by controlling the thermal decomposition of the carbonate catalyst, a crack-free working surface 23 of the carbonate PCD body is formed. Thus, in order to prevent or reduce thermal degradation of the PCD after HPHT sintering and during heat-treatment cycles below the threshold 1200° C. (ranging from temperatures between 1100° C.-1200° C.), various embodiments provide for a MgCO<sub>3</sub> carbonate catalyst that infiltrates the diamond particles during HPHT sintering and fully (or mostly) decomposes at a temperature below the 1200° C. threshold during subsequent heat-treatment cycles.

Generally, a carbonate catalyst such as MgCO<sub>3</sub> may begin to decompose at a temperature of approximately 400° C. at ambient pressure. The thermal decomposition temperature of MgCO<sub>3</sub> is related to the pressure. Thus, for example, MgCO<sub>3</sub> will remain in its major phase without fully decomposing when heat-treated after HPHT sintering for one hour under vacuum to a temperature of 1200° C., as shown in FIG. 6 and Table 1, below. FIG. 6 shows an X-ray diffraction pattern graph for a carbonate polycrystalline diamond layer including less than 0.2 wt % silicon, heat-treated to 1200° C. under vacuum. Table 1, interpreting the patterns displayed in FIG. 6, demonstrates an example including a MgCO<sub>3</sub> catalyst based carbonate PCD, where the carbonate PCD assembly includes less than 0.2 wt % Si (and/or Al) heat-treated to 1200° C. under vacuum. According to this example and the data shown in Table 1, approximately 35% of the carbonate catalyst entered the thermal decomposition phase, converting the carbonate catalyst (MgCO<sub>3</sub>) into an oxide (MgO) and releasing carbon dioxide (CO<sub>2</sub>). Thus, in the example in FIG. 6 and Table 1, where the carbonate PCD contained a mixture of 97.29 wt % diamond particles, less than 0.2 wt %

Si, and the remaining weight percentage a carbonate catalyst (MgCO<sub>3</sub>), heat-treated to 1200° C. under vacuum for one hour, approximately 0.97% of the approximately 2.71% of MgCO<sub>3</sub> converted to MgO. Accordingly, the addition of the MgCO<sub>3</sub> catalyst, according to the details of the example in FIG. 6 and Table 1, at the levels disclosed in Table 1, may not achieve full catalyst decomposition during a post-HPHT sintering heat-treatment temperature below a 1200° C. threshold.

TABLE 1

| Phase Content for FIG. 6 X-Ray Diffraction Pattern |         |                   |       |
|----------------------------------------------------|---------|-------------------|-------|
|                                                    | Diamond | MgCO <sub>3</sub> | MgO   |
| Content                                            | 97.29%  | 1.75%             | 0.97% |

However, by mixing the components of the first, second, and/or third layer including the carbonate PCD body before sintering with a Si and/or Al compound according to various embodiments disclosed herein, full thermal decomposition of the MgCO<sub>3</sub> carbon catalyst at a post-HPHT sintering heat-treatment temperature below 1200° C. may be realized. When the Si and/or Al compound mixed into the first, second, and/or third layer according to embodiments of the present disclosure reacts with the MgCO<sub>3</sub> catalyst, the result is the formation of MgSiO<sub>3</sub>, Mg<sub>2</sub>SiO<sub>4</sub>, MgAl<sub>2</sub>O<sub>4</sub> and/or combinations thereof. The compounds formed as a result of the reaction of the Si and/or Al compounds with the MgCO<sub>3</sub> promote thermal decomposition of the MgCO<sub>3</sub> at a lower temperature than the temperature of thermal decomposition under vacuum during heat-treatment cycles when Si and/or Al is/are not included. According to various embodiments, the MgCO<sub>3</sub> will enter the full thermal decomposition phase at or below the 1200° C. threshold for thermal degradation of the carbonate PCD, itself, and thus cause a reduction in the cracks often formed in the carbonate PCD at heat treatment cycles of temperatures between 800° C. and 1200° C. As shown in FIG. 7 and Table 2 below, in some embodiments the MgCO<sub>3</sub> of the carbonate PCD containing approximately 1.5 wt % Si, measured using energy dispersive spectroscopy (EDX), and heat-treated to 900° C. under vacuum, entered the full thermal decomposition phase converting to an oxide, MgSiO<sub>3</sub>, and Mg<sub>2</sub>SiO<sub>4</sub>, while the MgCO<sub>3</sub> of the carbonate PCD including with less than 0.2 wt % Si and heat-treated to 900° C. under vacuum did not enter the thermal decomposition phase, and remained in the MgCO<sub>3</sub> phase. In the embodiment of FIG. 7, the diamond particles of the first layer were mixed with 1% MgCO<sub>3</sub> and 0.5 wt % SiC, and the diamond particles of the second layer were mixed with 3% MgCO<sub>3</sub> and 0.5 wt % SiC. The assembly was infiltrated with a third layer containing MgCO<sub>3</sub> adjacent to the first layer. After HPHT sintering, the first layer had a thickness of approximately 2.0 mm, and the second layer had a thickness of approximately 6.0 mm, as shown in FIG. 8.

TABLE 2

| Phase Content for FIG. 7 X-Ray Diffraction Pattern |         |                   |       |                    |                                  |
|----------------------------------------------------|---------|-------------------|-------|--------------------|----------------------------------|
| Phase                                              | Diamond | MgCO <sub>3</sub> | MgO   | MgSiO <sub>3</sub> | Mg <sub>2</sub> SiO <sub>4</sub> |
| With <0.2 wt % Si                                  | 97.3%   | 2.7%              |       |                    |                                  |
| With ~1.5 wt % Si                                  | 96.8%   |                   | 0.45% | 1.38%              | 1.2%                             |

In some embodiments, by increasing the volume of MgCO<sub>3</sub> premixed with the diamond particles of the second layer, or as part of an additional third layer, thermal decomposition of the MgCO<sub>3</sub> at a lower temperature is promoted,

causing thermal decomposition under vacuum during heat-treatment cycles. The additional volume of  $\text{MgCO}_3$  results in the formation of larger pore channels during HPHT sintering, allowing the  $\text{CO}_2$  gas formed during subsequent thermal decomposition of the  $\text{MgCO}_3$  to more easily release from the PCD body. As shown in Table 3 below, in one embodiment, the phase ratio of  $\text{MgO}$  to  $\text{MgCO}_3$ , after heat-treating a carbonate PCD body under vacuum at a temperature of 1100° C. (after HPHT sintering), increases as the volume of  $\text{MgCO}_3$  premixed with the diamond particles or as part of a third layer is increased. In one embodiment including a 3% premixed volume of  $\text{MgCO}_3$ , the phase ratio is approximately 0.07, while in another embodiment including a 5% premixed volume of  $\text{MgCO}_3$ , the ratio increases to 1.63, and in another embodiment including a 7% premixed volume of  $\text{MgCO}_3$ , the ratio increases drastically to 13.85.

TABLE 3

| Phase Ratio After Heat Treating at 1100° C. for $\text{MgCO}_3$ PCD Measured by X-ray Diffraction |                                            |
|---------------------------------------------------------------------------------------------------|--------------------------------------------|
| Premixed Amount                                                                                   | Phase Ratio ( $\text{MgO}/\text{MgCO}_3$ ) |
| 3%                                                                                                | 0.07                                       |
| 5%                                                                                                | 1.63                                       |
| 7%                                                                                                | 13.85                                      |

However, an increase in the volume of  $\text{MgCO}_3$  premixed into a layer, while promoting thermal decomposition of the catalyst at a lower temperature, can also decrease the wear resistance of the PCD body surface as a result of the formation of larger pore channels on the surface and also result in a decrease in diamond density. Accordingly, in various embodiments, the increased volume of  $\text{MgCO}_3$  is only added to the second layer, or as part of the additional third layer, while a first layer, which will form a working surface of the carbonate PCD, includes a comparably decreased volume of  $\text{MgCO}_3$  where the working surface is created. As a result of the increased volume of  $\text{MgCO}_3$  premixed into the second and/or third layers, these layers will be generally thicker than the first layer, which contains a lesser quantity of the  $\text{MgCO}_3$  premixed into the layer. Accordingly, the  $\text{MgCO}_3$  catalyst in the second layer, which will be heat-treated after HPHT sintering, will be more fully decomposed at a lower temperature than the  $\text{MgCO}_3$  catalyst in the first layer. The result of this variance in thermal decomposition properties of the layers is that the carbonate PCD will form minimal to no cracks during subsequent heat-treatment cycles because the  $\text{CO}_2$  decomposed from the first layer including the working surface can be quickly released through the thinner layer first layer, rather than remain trapped inside the thicker second and/or third layers. Since Si and/or Al compounds are not catalysts, in order to decrease wear resistance, the amount of these compounds that accumulates on the working surface should be minimized. For this reason, infiltrating the first layer at the working surface side with additional  $\text{MgCO}_3$  catalyst, for example, by placing the third layer or another fourth layer of  $\text{MgCO}_3$  catalyst adjacent to the first layer so that the first layer is sandwiched between the third layer, or the fourth layer, and the second layer, allows for the formation of the working surface with minimal or reduced cracks, while maintaining wear resistance at the working surface.

A method for forming the carbonate PCD body with a distribution of Si and/or Al elements is shown in FIG. 4 with additional reference to FIGS. 2a-2d, according to one

embodiment. The method includes placing a first layer 22 of diamond particles mixed with a first quantity of a carbonate catalyst having a first percentage by weight for forming a working surface 21 of the carbonate PCD body 20 (block 101). In some embodiments, the first percentage by weight of the carbonate catalyst is approximately 1.0 wt % (based on the weight of the first layer). In some embodiments, the first percentage by weight of the carbonate catalyst is approximately 0.5-3.0 wt % (based on the weight of the first layer) and the first layer has a thickness of approximately 1-3 mm. The method then includes placing a second layer 24 of diamond particles mixed with a second quantity of a carbonate catalyst having a second percentage by weight, adjacent to the first layer 22, for forming a non-working surface 21 of the carbonate PCD body (block 102). The second layer 24 includes a second percentage by weight of the carbonate catalyst that is greater than the first percentage of the first layer 22, such that the non-working surface 21 contains a greater carbonate catalyst composition than the working surface 22. As a result of the reduced quantity of the carbonate catalyst compound at the first layer or working surface 22, in most embodiments, the first layer 22 is infiltrated from the working surface 23 with an additional layer of carbonate catalyst prior to HPHT sintering. Thus, in some embodiments, the first layer 22 can include multiple layers, including a layer of carbonate catalyst adjacent to the working surface side 23 of the first layer 22. In some embodiments, the second percentage of the carbonate catalyst is greater than 1.0 wt % (based on the weight of the second layer). In some embodiments, the second percentage of the carbonate catalyst is 5.0 wt % (based on the weight of the second layer). In some embodiments, the second percentage of the carbonate catalyst is 7.0 wt % (based on the weight of the second layer). In some embodiments, the second percentage by weight of the carbonate catalyst is approximately 2.0-9.0 wt % (based on the weight of the second layer) and the second layer has a thickness of approximately 3-15 mm. In some embodiments, the first layer has a first percentage of the carbonate catalyst that is greater than 1.0 wt % (based on the weight of the first layer).

The method includes introducing a Silicon (Si) and/or Aluminum (Al) compound at the second layer 24 (block 103). In various embodiments, this Si and/or Al compound includes Al, Si,  $\text{SiO}_2$ ,  $\text{Al}_2\text{O}_3$ , SiC,  $\text{Al}_3\text{C}$ , and/or combinations thereof. In some embodiments, the Si and/or Al compound is Si included at about 1.5 wt %. In some embodiments, the Si and/or Al is included in the carbonate catalyst at about 1.5 wt % based on the weight of the carbonate catalyst. In other embodiments, the Si and/or Al is SiC included at 0.5 wt % (e.g., based on the weight of the layer it is in). The Si and/or Al compound can be combined directly with the second layer forming a mixture of diamond particles, mixed with the second percentage of carbonate catalyst, and mixed with the Si and/or Al compound for forming the second layer 24. In another embodiment, the Si and/or Al compound is applied in a separate third layer 26 adjacent to the second layer 24, and disposed at an opposite surface from the first layer working surface 23, and adjacent to the non-working surface 21, as, for example, shown in FIGS. 2b and 2d. In some embodiments, the third layer 26 also includes a third percentage by weight of the carbonate catalyst combined with the Si and/or Al compound. In some embodiments, the Si and/or Al compound is  $\text{SiO}_2$  included at 1.5% wt in the third layer. In another embodiment, the Si and/or Al compound can be combined directly with the first layer of diamond particles mixed with the first percentage of carbonate catalyst to form the first layer 22 or working

surface 23. In other embodiments, the Si and/or Al compound can be combined directly with the additional layer of carbonate catalyst placed adjacent to the working surface 23 side of the first layer 22 prior to HPHT sintering. In other embodiments, the second layer 24 can include multiple layers, including layers of varying compositions, catalyst types and volumes, and/or thicknesses.

In another embodiment, as shown in FIGS. 2c and 2d, a substrate is provided adjacent to the second layer 24 (FIG. 2c) or adjacent to an optional third layer 26 (FIG. 2d), or adjacent to the non-working surface 21 of the second layer 24. The substrate bonds to the non-working surface during HPHT sintering. The substrate is useful for attaching the carbonated PCD body to a cutting tool. The substrate may also provide a source of a solvent metal catalyst, such as cobalt, for HPHT sintering. The substrate can be selected from the group including metallic materials, ceramic materials, cermet materials, and combinations thereof. Examples include carbides such as WC, W 2 C, TiC, VC, and SiC. In some embodiments, the substrate is formed of cemented tungsten carbide.

With reference again to FIG. 4, after placing the series of layers 22, 24, and optionally 26 and/or substrate 27, the method includes subjecting the refractory can or container 28 including the series of layers to HPHT sintering (block 104). In some embodiments, the first layer 22 includes an additional layer of carbonate catalyst adjacent to its working surface 23 side. The method includes HPHT sintering the carbonate PCD body according to various embodiments to a temperature greater than 1350° C. and a pressure of about or greater than 5 GPa or 50 kbar. In some embodiments, the method includes HPHT sintering the carbonate PCD to a temperature greater than 1800° C. and a pressure of about or greater than 6.5 GPa or 65 kbar. At this HPHT sintering temperature, the carbonate catalyst at each layer melts, entering the liquid phase, and infiltrating into the diamond particles of the first and second layers, bonding the diamond particles grains together to form the carbonate PCD (block 105), as also shown in FIG. 3a. Also, at this HPHT sintering temperature, most of the Si and/or Al compounds, including SiC and/or Al<sub>2</sub>O<sub>3</sub> will react with the carbonate catalyst to form a liquid. The liquid will flow in the general direction of liquid flow, from the surface where it was deposited to the opposite surface (block 105). In some embodiments, where the Si and/or Al compound is directly mixed with the particles and catalyst of the second layer or a separate third layer adjacent to the second layer prior to HPHT sintering, the Si and/or Al rich liquid flows toward the first layer or working surface after HPHT sintering. In another embodiment, the Si and/or Al compound is directly mixed with the particles and catalyst of the first layer prior to HPHT sintering, and the Si and/or Al rich liquid flows toward the second layer or non-working surface after HPHT sintering. As a result of the differential volumes of carbonate catalyst at each of the first and second layers, and as a result of the flow of the Si and/or Al rich liquid after HPHT sintering to the opposite surface from its disposition location prior to HPHT sintering, the working surface and non-working surface sides of the carbonate PCD body have different thermal decomposition behaviors. Some portion of the Si and/or Al compound may remain in the layer in which it was introduced.

By way of example, FIG. 8 shows the distribution of Si along the thickness of a PCD body after HPHT sintering according to some embodiments including 0.5 wt % SiC. As shown in FIG. 8, the entire PCD body has a thickness of approximately 8 millimeters (mm) as measured from the

non-working surface. The SiC compound was originally mixed in with the diamond particles and MgCO<sub>3</sub> catalyst at both the first layer and the second layer. In this example, the first layer diamond particles were mixed with 1 wt % MgCO<sub>3</sub> and 0.5 wt % SiC, and the second layer diamond particles were mixed with 3 wt % MgCO<sub>3</sub> and 0.5 wt % SiC. A layer of MgCO<sub>3</sub> was also introduced at the working surface side of the first layer to infiltrate the first layer with MgCO<sub>3</sub>. During HPHT sintering, the SiC compound reacted and melted, and the resulting Si liquid flowed to the opposite surface across the 8 mm thickness of the PCD body, mostly accumulating at a depth between 0.0 mm to 4.0 mm, where the depth measured from the non-working surface side is 8.0 mm, and from the non-working surface side is 0.0 mm. After sintering, the first layer had a thickness of approximately 2.0 mm, and the second layer had a thickness of approximately 6.0 mm.

By way of example, FIG. 9 shows another example of the distribution of Si along the thickness of a PCD body after HPHT sintering according to another embodiment including a SiO<sub>2</sub> compound. In this example, the diamond particles of the first layer were mixed with 1 wt % MgCO<sub>3</sub> and 1.5 wt % SiO<sub>2</sub> (e.g., the SiO<sub>2</sub> being 1.5 wt % of the MgCO<sub>3</sub>), while the diamond particles of the second layer were mixed with 5 wt % MgCO<sub>3</sub> and 1.5 wt % SiO<sub>2</sub> (e.g., the SiO<sub>2</sub> being 1.5 wt % of the MgCO<sub>3</sub>). A layer of MgCO<sub>3</sub> was also introduced at the working surface side of the first layer to infiltrate the first layer with MgCO<sub>3</sub>. After HPHT sintering, the first layer had a thickness of approximately 2.5 mm (where the first layer is shown in FIG. 9 ranging from 11.5 mm to 14 mm in depth) and the second layer had a thickness of approximately 11.5 mm (where the second layer is shown in FIG. 9 ranging from 0 mm to 11.5 mm in depth). As a result of the SiO<sub>2</sub> infiltrated in the MgCO<sub>3</sub>, a non-uniform Si distribution was detected after HPHT sintering. However, most of the Si element accumulated along the non-working surface area close to the working surface layer.

By way of example, FIG. 10 shows another example of the distribution of Si along a thickness of a PCD body after HPHT sintering, showing an embodiment where the additional layer of MgCO<sub>3</sub> layer was introduced at the working surface side, and an embodiment where the additional MgCO<sub>3</sub> layer was introduced at the non-working surface side. The diamond particles of the first layer were mixed with 1 wt % MgCO<sub>3</sub> and the first layer had a thickness of approximately 2 mm, and the diamond particles of the second layer were mixed with 3 wt % MgCO<sub>3</sub> and the second layer has a thickness of approximately 6 mm. One sample is infiltrated with MgCO<sub>3</sub> from working surface side and another one from non-working surface side. The resulting Si distribution is different at each embodiment. When the MgCO<sub>3</sub> layer infiltrated from the working surface side, the Si level was high at non-working surface side, but where the MgCO<sub>3</sub> layer infiltrated from the non-working surface side, the Si level was high at the working surface side. To improve the wear resistance at the working surface side, thus, the MgCO<sub>3</sub> layer may be infiltrated from the working surface side.

In some embodiments, where the Si and/or Al compound is directly mixed with the particles and catalyst of the second layer or includes a separate third layer adjacent to the second layer prior to HPHT sintering, the resulting carbonate PCD after HPHT sintering has a first layer or working surface with a higher concentration of the Si and/or Al compound. And, as a result of the first layer including the working surface having a percentage of the carbonate catalyst less than that of the second layer prior to HPHT sintering, a

## 11

greater percentage of the carbonate catalyst may be thermally decomposed at the first layer working surface, than at the second layer or non-working surface, during heat-treatment cycles. The higher concentration of the Si and/or Al compound formed at the first layer including the working surface results in a lower thermal decomposition temperature for the carbonate catalyst than there would be otherwise without the Si and/or Al compound at the working surface than throughout the remainder of the carbonate PCD, including throughout the second layer. In other embodiments, the decomposition temperature of the first layer may be lower than, equal to, or even greater than the decomposition temperature of the second layer, as a result of the Si and/or Al compound introduced prior to HPHT sintering, however, the resulting thermal decomposition temperature of the first layer will be less than the thermal decomposition temperature for the carbonate catalyst not including a Si and/or Al compound.

In some embodiments, a diamond compact includes a carbonate PCD body with a distribution of Si and/or Al elements. A diamond compact 30 according to some embodiments is shown in FIGS. 3a and 3b. The diamond compact 34 includes a carbonate PCD body with a first section having a first layer 22 including a working surface 23, a second layer 24 including a non-working surface, and an optional substrate 27 (shown in FIG. 3b). The diamond compact 34 according to various embodiments is more thermally stable, and is able to operate at elevated temperatures without experiencing cracking caused from the thermal decomposition of the PCD during heat treatment cycles between 800° C. and 1200° C.

The diamond compact 30 shown in FIGS. 3a and 3b is formed as a cutting element for incorporation into a cutting tool. FIG. 5 shows a drag bit 40 incorporating the cutting element of FIG. 3a or 3b, according to embodiments of the disclosure. The drag bit 40 may include several cutting elements 30 that are each attached to blades 32 that extend along the drag bit. The drag bit may be used for rock drilling operations. In other embodiments, other types of drilling or cutting tools incorporating cutting elements (e.g., that have a thermally stable diamond element) forming at least a portion of the cutting edge of the cutting element, such as, for example, rotary or roller cone drilling bits, or percussion or hammer drill bits may be utilized. In some embodiments, the cutting element is a shear cutter.

In other embodiments, rather than the carbonate catalyst, and/or the Si and/or Al compounds being mixed in or pre-mixed with the diamond particles of the first layer, and/or the second layer, the carbonate catalyst and/or the Si and/or Al compounds may be applied as separate layer(s) adjacent to the first layer or the second layer, or any other layer including diamond particles. The separate layer(s) including the carbonate catalyst and/or the Si and/or Al compounds may then infiltrate into the corresponding adjacent layer during HPHT sintering.

Although only a few embodiments have been described in detail above, those skilled in the art will readily appreciate that many modifications are possible in the embodiments without materially departing from this disclosure. Accordingly, all such modifications are intended to be included within the scope of this disclosure. It is the express intention of the application not to invoke 35 U.S.C. §112, paragraph 6 for any limitations of any of the claims herein, except for those in which the claim expressly uses the words 'means for' together with an associated function.

## 12

What is claimed is:

1. A carbonate polycrystalline diamond body having a working surface opposite a non-working surface, the carbonate polycrystalline diamond body comprising:
  - 5 a first layer comprising a material microstructure comprising a plurality of bonded-together diamond crystals and interstitial spaces therebetween, a portion of the interstitial spaces being occupied by a first concentration of magnesium, the first layer defining the working surface, wherein at least a portion of the magnesium is in the form of magnesium carbonate;
  - 10 a second layer adjacent to the first layer at a location opposite the working surface, the second layer comprising a material microstructure comprising a plurality of bonded-together diamond crystals and interstitial spaces therebetween, a portion of the interstitial spaces being occupied by a second concentration of magnesium greater than the first concentration, wherein at least a portion of the magnesium is in the form of magnesium carbonate; and
  - 15 a quantity of at least one of silicon, aluminum, or a combination thereof in at least one of the first layer or the second layer.
2. The carbonate polycrystalline diamond body of claim 1, wherein the first layer comprises a majority of the quantity of the silicon, aluminum, or a combination thereof.
3. The carbonate polycrystalline diamond body of claim 1, wherein the second layer comprises a majority of the quantity of the silicon, aluminum, or a combination thereof.
4. The carbonate polycrystalline diamond body of claim 1, wherein the carbonate polycrystalline diamond body is formed by high pressure high temperature sintering.
5. The carbonate polycrystalline diamond body of claim 4, wherein the first layer is formed by mixing a first quantity of diamond particles with a first volume percentage of magnesium carbonate, and the second layer is formed by mixing a second quantity of diamond particles with a second volume percentage of magnesium carbonate greater than the first volume percentage of magnesium carbonate and with the quantity of at least one of silicon, aluminum, or a combination thereof.
6. The carbonate polycrystalline diamond body of claim 5, wherein the high pressure and high temperature sintering causes the quantity of at least one of silicon, aluminum, or a combination thereof, of the second layer to flow in a direction toward the first layer, forming a non-uniform distribution of the at least one of silicon, aluminum, or a combination thereof, wherein the majority of the at least one of silicon, aluminum, or a combination thereof, is in the first layer, and the resulting carbonate polycrystalline diamond body has a working surface with a different thermal decomposition behavior than the non-working surface.
7. The carbonate polycrystalline diamond body of claim 5, wherein the at least one of silicon, aluminum, or a combination thereof, includes at least one selected from the group consisting of aluminum, silicon, silicon dioxide, aluminum oxide, silicon carbide, neutral carbon aluminum cluster, and combinations thereof.
8. The carbonate polycrystalline diamond body of claim 1, wherein the carbonate polycrystalline diamond body further comprises a substrate adjacent to the second layer opposite the first layer.
9. The carbonate polycrystalline diamond body of claim 1, wherein the quantity of silicon in at least the first layer or the second layer is less than 1.5 wt % based on the total weight of the layer the silicon is in.

**13**

**10.** The carbonate polycrystalline diamond body of claim 1, wherein the first and second layers comprise magnesium in the form of materials selected from the group consisting of MgCO<sub>3</sub>, MgSiO<sub>3</sub>, Mg<sub>2</sub>SiO<sub>4</sub>, MgAl<sub>2</sub>O<sub>4</sub>, and combinations thereof. <sup>5</sup>

**11.** The carbonate polycrystalline diamond body of claim 1, further comprising a third concentration of magnesium to form a third layer adjacent to the first layer, such that the first layer is sandwiched between the third layer and the second layer. <sup>10</sup>

**12.** The carbonate polycrystalline diamond body of claim 1, wherein the second layer comprises large pore channels.

\* \* \* \* \*

**14**